# EUROPEAN PATENT SPECIFICATION

(11) **EP 0 055 377 B1**
(45) Date of publication and mention of the grant of the patent: **10.04.1985**
(21) Application number: 81109163.6
(22) Date of filing: 29.10.1981
(51) Int. Cl.: C25D 3/56, H01F 10/14

(54) **Method of depositing nickel-iron-boron alloy magnetic films**
Verfahren zum Abscheiden magnetischer Filme aus einer Nickel-Eisen-Bor-Legierung
Procédé de dépôt de films magnétiques à base de nickel-fer-bore

(30) Priority: 31.12.1980 US 221598
(43) Date of publication of application: 07.07.1982
(73) Proprietor: International Business Machines Corporation, Armonk, N.Y. 10504 (US)
(72) Inventor: Blakeslee, Marybelle Capron, Golden Colorado 80401 (US); Olsen, Judith Diane, Golden's Bridge New York 10526 (US); Romankiw, Lubomyr Taras, Briarcliffe Manor New York 10510 (US)
(74) Representative: Hobbs, Francis John

## Description

This present invention relates to methods of depositing nickel-iron-boron alloy magnetic films.

U.S. patent specification 3,483,029 entitled "Method and Composition for Depositing Nickel-iron-Boron Magnetic Films" describes in the Example, the electroless deposition of an alloy film containing 0.8% B, 19.3% Fe and the remainder Ni, from a bath containing a borane reducing agent (dimethylamine borane). The film was 1.255 pm (12,550 A) thick and had a coercivity of Hₒ=1.0 e. The magnetostriction was near zero. The anisotropic field was about 4.8 Oe. The pH of the bath was above 8.

A process for depositing a nickel-iron-boron alloy magnetic film containing 0.1 to 2 per cent boron by weight, 17 to 27 per cent iron by weight and the balance nickel, the process employing a bath containing a borane reducing agent, is characterised according to the invention, by being an electrolytic deposition process employing a bath having a pH at or below 2.5.

Preferably, the borane reducing agent is dimethylamine borane. The bath may also contain a pH regulator, a surfactant and sodium saccharin.

The alloy film deposited by a process in accordance with the invention can be at least 0.3 µm (3000 A) thick and have a coercivity less than 0.1 oersted (n/25 ampere turns per cm).

The present invention provides nickel-iron-boron alloy magnetic films having extremely low coercivity and very high resistance to corrosion. Magnetic films 3000 A thick or thicker deposited according to the present invention, have a coercivity and a bubble collapse field of less than 0.1 Oe (n/25 ampere turns per cm). They also have excellent magnetic anisotropy.

In accordance with the present invention, magnetic films are electrodeposited from an acid (pH at or below 2.5) bath containing small amounts of a boron reducing agent such as dimethylamine borane.

Table I below gives one specific bath formulation and a range of bath formulations.

The dimethylamine borane (DMAB) is predissolved in 100 cc H₂0. 1.6 g/I of DMAB is near maximum solubility in the specific bath in Table I. The sodium lauryl S0₄ is a surfactant, which improves plating. The sodium saccharin serves to reduce stress in the plated film. The boric acid serves as a pH regulator and deposit brightener.

λ=0 at 16.5 mA/cm² when FeCl₂ · 4H₂0=1.9 g/l. Agitation rate anywhere from 0.5 cycle per second to 2 cycles per second can be utilized. Agitation of 1 cycle/second in a paddle cell is the equivalent of 200 rpm on a rotating disc electrode.

After the addition of DMAB solution to the bath, the pH rises for a few minutes. After readjusting the pH to 2.5 the bath is usable. If the concentration of FeCI₂ . 4H₂0 is higher than 1.9 g/I, the currentwill have to be raised in order to maintain the λ=0 composition. For example, if the FeCl₂ · 4H₂O is increased to 5.0 g/l, λ=0 is obtained at 49.6 mA/cm² when plating onto a cathode in a continuous sheet form. At this high current density the DMAB seems to have a smaller effect on the film. When plating is conducted at low density, the resulting films incorporate 2% boron. Despite this small quantity of boron, the magnetic behaviour of the film is markedly improved. The films also have excellent anisotropy.

A NiFeB film 0.54 µm (5400 Å) thick deposited in accordance with the present invention on a substrate comprising 0.1 pm (1000 Å) platinum 0.01 µm (100 Å) titanium on glass had a value for Hₒ of 0.1 Oe (n/25 ampere turns per cm) or less. The instrument commonly used to measure the magnetic properties of NiFe films is not sufficiently sensitive to measure values at this very low level.

When NiFeB films are deposited in accordance with the present invention on T and I bars, or when a sheet film is shaped by ion milling or sputter etching, the superiority in coercivity of NiFeB over NiFe is still apparent. This makes the NiFeB quite useful for bubble memory applications. When plating through masks, we have also discovered to our surprise that the deposits of NiFeB are smoother and the thickness of individual features over a large area are considerably more uniform than for NiFe. This suggests that in addition to providing boron incorporated in the film, DMAB acts as a smoothing agent and a levelling agent.

While the above example employed dimethylamine borane, it should be apparent to those skilled in the art that other borane containing compounds, particularly borane reducing agents, may be used to obtain similar results. Other useful compounds include, for example, amine boranes such as trimethylamine borane, and other aliphatic heterocyclic, arylamine and heteroaromatic boranes and borohydrides.

### I Examples of films plated onto a continuous sheet metal cathode

Films were electroplated at room temperature in a >40 Oe magnetic field from the bath as shown in Table I onto a cathode in a continuous sheet form except for the following changes:
(a) FeCl₂ · 4H₂O was 1.6 g/l
   DMAB 1.2 g/I
   and current density was 5.0 mA/cm²

The resulting 0.4 pm (4000 Å) thick film had a coercivity Hₒ<0.1 Oe (π/25 ampere turns per cm) and a very square B-H loop. The film composition was 19% Fe, 0.6% B, 80.2% Ni. The film was zero magnetostrictive (λ=0).
(b) FeCl₂ · 4H₂O was 1.8 g/l
   DMAB was 1.5 g/I
   current density was 10 mA/cm²

The composition of the 0.4 µm (4000 A) film was 19.4% Fe, 0.4% B and 80.2% Ni. Magnetic results were substantially the same as in (a) above.
(c) FeCl₂ · 4H₂O was 1.8 g/l
   DMAB was 1.5 g/I
   current density was 21.6 mA/cm²

The composition of the 4000 A film was 21.6% Fe, 0.3% B and 78.1% Ni. Magnetic properties were substantially the same as in (a) above. Film was slightly off from zero magnetostriction.

### II Examples of films plated through photoresist masks

(a) Discrete features were plated onto a continuous thin metallizing starter sheet cathode on top of a garnet coated with 0.3 µm (3000 Å) of SiO₂ spacer and on top of Si wafer with 0.3 µm (3000 Å) Si0₂ masked by Shipley 1350 resist with 2 µm wide features exposed in resist to define the bubble memory C- and I-bar and chevron pattern.

The bath composition was:

the overall current density id varied from 3.48 to 5 mA/cm².

The film compositions were:

In both cases where the DMAB was added to the solution the films were smoother; the thickness of various features showed less variation from spot to spot on the wafer; the coercive force of the features was much lower than in the features plated without the Boron, and the garnet devices showed lower operative margins of the magnetic field. The operative margin was much lower than in devices plated in the absence of DMAB in the bath (a). When DMAB was added (baths (b) and (c)), the percentage of iron in the features, plated through a mask, was always higher than in the absence of DMAB.

(b) Discrete features were plated onto a continuous thin film metallizing starter sheet on Si0₂ on a garnet and on 0.3 µm (3000 Å) of SiO₂ on Si wafers through 2 pm openings in Shipley 1350 resist.

The bath composition was:

Overall current density varied from 5 to 7.0 mA/cm².

Film compositions were:

Films were plated 0.35 µm (3500 Å) thick.

In all cases the films have shown superior surface smoothness, superior uniformity of thickness from feature to feature, very low closed loop coercive force and the bubble devices plated on garnets operated at much lower minimum operating bias field.

The minimum bias field in the absence of the Boron in the 3500 A film plated in 2 µm wide features is of the order of 25 to 30 Oe, while for the same thickness film plated from the above bath containing Boron the minimum bias field is consistently 15 Oe or lower.

(c) Discrete features were plated onto a continuous thin film metallizing starter sheet on Si0₂ on a garnet and on 0.3 µm (3000 Å) Si0₂ on top of Si wafers through 2 µm openings of the C- and I-Bar bubble pattern in Shipley 1350 resist mask.

The bath composition was:

overall current density id varied from 3.6 to 7.2 mAlcm².

The resulting 0.35 pm (3500 A) plated features had the following characteristics:

All films in which DMAB was used showed superior smoothness, superior thickness uniformity from feature to feature and superior magnetic characteristics. The bubble memory devices plated with these films on garnet showed much lower value of the lower operating margin of the bubble devices.

Corrosion testing of all films plated from the bath containing DMAB, and hence containing B in addition to Ni and Fe, showed 4 to 10 times higher corrsion resistance than the films plated from the above bath in absence of DMAB.

## Claims

1. A process for depositing a nickel-iron-boron alloy magnetic film containing 0.1 to 2 per cent boron by weight, 17 to 27 per cent iron by weight and the balance nickel, the process employing a bath containing a borane reducing agent, characterised by the process being an electrolytic deposition process employing a bath having a pH at or below 2.5.

2. A process as claimed in claim 1, in which the borane reducing agent is dimethylamine borane.

3. A process as claimed in claim 1 or claim 2, in which the bath also contains a pH regulator, a surfactant and sodium saccharin.

4. A magnetic film deposited by a process as claimed in any preceding claim, the film being at least 0.3 pm (3000 Å) thick and having a coercivity less than 0.1 oersted (π25 ampere turns per cm).

## Revendications

1. Un procédé pour déposer un film magnétique en alliage de nickel-fer-bore contenant 0,1 à 2 pour cent de bore en poids, 17 à 27 pour cent de fer en poids et le reste en nickel, ce procédé employant un bain contenant un agent réducteur de borane caractérisé par le traitement qui est un procédé de dépôt électrolytique employant un bain dont le pH est égal ou inférieur à 2,5.

2. Un procédé conforme à la revendication 1, dans lequel l'agent réducteur de borane est du diméthylamine borane.

3. Un procédé conforme à la revendication 1 ou 2, dans lequel le bain contient également un régulateur de pH, un surfactant et de la saccharine de sodium.

4. Un film magnétique déposé par un procédé conforme à l'une quelconque des revendications précédentes, le film étant épais d'au moins 0,3 pm et ayant une coercivité inférieure à 0,1 Oersted (n/25 ampères/tours par cm).

## Patentansprüche

1. Verfahren zur Abscheidung eines magnetischen Films aus einer Nickel-Eisen-Borlegierung mit 0,1 bis 2 Gewichtsprozent Bor, 17 bis 27 Gewichtsprozent Eisen und Rest Nikkel, wobei das Verfahren ein ein Boranreduktionsmittel enthaltendes Bad verwendet, dadurch gekennzeichnet, daß das Verfahren eine elektrolytische Abscheidung ist, welche ein Bad mit einem pH-Wert bei oder unter 2,5 verwendet.

2. Verfahren nach Anspruch 1, bei welchem das Boranreduktionsmittel Dimethylaminboran ist.

3. Verfahren nach Anspruch 1 oder 2, bei welchem das Bad einen pH-Wert-Regier, ein oberflächenaktives Mittel und Natriumsaccharin enthält.

4. Nach einem Verfahren gemäß irgendeinem der vorstehenden Ansprüche abgeschiedener magnetischer Film, welcher wenigstens 0,3 µm (3000 Å) dick ist und eine Koerzitivfeldstärke von weniger als 0,1 Oersted (n/25 Amperewindungen pro cm) hat.
